# EUROPEAN PATENT SPECIFICATION

(11) **EP 1 853 750 B1**
(45) Date of publication and mention of the grant of the patent: **20.04.2011**
(21) Application number: 05851693.1
(22) Date of filing: 14.11.2005
(51) Int. Cl.: C25D 11/24, C23C 22/34, C23C 22/83

(54) **PROCESS FOR SEALING PHOSPHORIC ACID ANODIZED ALUMINUMS**
VERFAHREN ZUM VERSIEGELN VON MIT PHOSPHORSÄURE ANODISIERTEM ALUMINIUM
PROCEDE D'ETANCHEIFICATION D'ALUMINIUM ANODISE A L'ACIDE PHOSPHORIQUE

(30) Priority: 15.02.2005 US 58533
(43) Date of publication of application: 14.11.2007
(73) Proprietor: The United States of America, as represented by The Secretary of the Navy, et al., Patuxent River, MD 20670-1550 (US)
(72) Inventor: MATZDORF, Craig, A., California, Maryland 20619 (US); NICKERSON, William, C., Jr., Patuxent River, Maryland 20670 (US); BECK, Erin, N., Patuxent River, Maryland 20670 (US)
(74) Representative: Winter, Konrad Theodor
(86) International application number: PCT/US2005/041425
(87) International publication number: WO 2006/088520

(56) References cited:
- EP-A- 1 378 585
- US-A- 4 084 014
- US-A- 4 467 028
- US-A- 4 467 028
- US-A- 4 786 336
- US-A- 5 304 257
- US-B1- 6 663 700
- US-B1- 6 663 700
- US-B2- 6 511 532
- US-B2- 6 511 532

## Description

### ORIGIN OF INVENTION

The invention described herein was made by employee(s) of the United States Government and may be manufactured and used by or for the Government for governmental purposes without the payment of any royalties thereon or therefor.

### BACKGROUND OF THE INVENTION

US 6663700 relates to aqueous compositions and a process for post-treating metal coated substrates to provide colour recognition, and improve the corrosion-resistance, abrasion, and adhesion properties, comprising treating the metal coated substrates with an acidic aqueous solution containing a water soluble trivalent chromium compound.

EP 1378585 discloses a composition as well as a process for preparing a corrosion-resistant trivalent chromium coating on metal substrates comprising treating the substrates with an acidic aqueous solution, which is free of hexavalent chromium, comprising a water soluble trivalent chromium compound, a water soluble fluoride compound, and an additive for improved corrosion resistance properties.

US 5304257 relates to a process for preparing a corrosion-resistant trivalent chromium coating on aluminium and aluminium-alloy substrates (anodized or not) which comprises treating said substrates with an acidic aqueous solution free of hexavalent chromium and contains a trivalent chromium compound, a fluoride compound and a sufficient amount of an alkaline reagent to maintain the aqueous solution at a pH ranging from about 4,0 to 5,5 to form the trivalent chromium coating on said aluminium substrates.

US 4084014 discloses a process for sealing porosities of a surface layer of aluminium oxide formed by anodic oxidation on an article comprised of aluminium (or anodized aluminium) which comprises contacting said surface layer with an aqueous solution which includes phosphate ions, trivalent chromium ions, an organic resin and may also include zinc.

US 6511532, which is considered as the closest prior art, describes a composition as well as a process for post-treating anodized aluminium and anodized aluminium alloys to improve the corrosion-resistance, abrasion, and adhesion bonding properties which comprises sealing the anodized aluminium and aluminium alloys with an acidic aqueous solution which contains a water soluble trivalent chromium salt, however, without the addition of a divalent zinc compound.

### FIELD OF THE INVENTION

This invention relates to a process for depositing a film or coating onto aluminum and its alloys that have been phosphoric acid anodized. The coating system comprises phosphoric acid anodize aluminums, a supplemental post-treatment or seal coating, optimally, an adhesive bond primer or other supplemental coatings. Phosphoric acid anodized aluminum coatings are very porous and therefore have poor inherent corrosion resistance. These coatings do, however, have excellent adhesive properties. Accordingly these anodized coatings would benefit from a post-treatment or seal coating that enhances corrosion protection without adversely affecting the adhesion properties. The performance characteristics of this invention allows the phosphoric acid anodized coatings to be used in unpainted applications which are currently unfeasible; to replace chromic acid anodize aluminum and FPL Etch, both of which contain chromates for corrosion-prone fatigue-sensitive applications; in all adhesive bonding applications where the transition to non-chomated bond primers is made; and, in general use applications to reduce fatigue debit and coating weight compared to other general use anodize coatings.

This invention relates to a process for treating phosphoric acid anodized aluminum(s) to maintain and improve the corrosion-resistant properties. More specifically, this invention relates to the process of sealing phosphoric acid anodized aluminum and anodized aluminum alloys. The trivalent chromium post-treatment (TCP) process comprises an acidic aqueous solution containing effective amounts of at least one water-soluble trivalent chromium compound, an alkali metal hexafluorozirconate, at least one alkali metal tetrafluoroborate and/or hexafluorosilicate, at least one divalent zinc compound, and effective amounts of water-soluble thickeners and/or water-soluble surfactants.

Anodized aluminum(s) are generally sealed or post-treated after anodizing by processes employing a variety of sealing processes and compositions. Current high-performance post treatments or sealers for anodized aluminum are based on hexavalent chromium chemistry. Hexavalent chromium is highly toxic and a known carcinogen. As a result, the solutions used to deposit these protective coatings and the coating per se are toxic. These films or coatings do, however, yield good adhesion and improved corrosion resistance to the anodized aluminum. Typically, seal coatings are deposited onto the anodized coating at elevated temperatures and are usually applied by immersion or spray processes. Post treatments can be required by the military and by commercial specifications that govern each coating being treated. As such, there is not a unique "post treatment" specification for all anodize aluminums like there is for "conversion coating" aluminum.

Further, environmental laws, executive orders, and local occupational, safety, and health (OSH) regulations are driving the military and commercial users in the search for hexavalent chromium-free treatments. In the case of anodized aluminum, the anodize film and base metal are relatively non-toxic. With the addition of the required hexavalent chromium treatment, these coatings become toxic. While some other compositions used for coating anodized aluminum may not contain hexavalent chromium, their technical performance is inferior to the hexavalent chromium-based coatings. In addition, the use of hexavalent chromium-treatments is becoming more expensive as regulations tighten. Costs may become prohibitive with future restrictions imposed by the EPA. Thus, while existing hexavalent chromium-treatments are outstanding in their technical performance in that they provide enhanced corrosion protection and adhesion bonding e.g. with coatings such as paint at a low application cost, from a life-cycle cost, environmental, and OSH perspective, hexavalent chromium coatings are detrimental to both people and the environment.

In regard to adhesive bonding, phosphoric acid anodize is being implemented as an alternative to chromic acid anodize. Phosphoric acid anodize coatings provide excellent adhesive bonding performance, but fail to adequately protect the base aluminum from corrosion. While anodize sealers are typically applied to various other anodize coatings to boost corrosion performance, they are generally not applied to phosphoric acid anodize coatings because the adhesive bonding performance is significantly reduced. As a result, the corrosion protection of a phosphoric acid anodized coating is provided by chromated bond primers or general use primers. Phosphoric acid anodize coatings are characteristically columnar and porous, thus promoting excellent adhesive bonding performance. However, the columnar, porous structure also promotes corrosion making phosphoric acid anodize coatings particularly difficult to protect against corrosion. For example, phosphoric acid anodized "honeycomb" core, commonly used in military aircraft, corrodes quickly in service when its protective coating is damaged and would greatly benefit from a corrosion protective sealer that does not adversely impact the adhesive bonding characteristics of the anodize coating.

### SUMMARY OF THE INVENTION

This invention relates to a process of post-treating or sealing phosphoric acid anodized aluminum and its alloys at ambient temperatures or higher e.g. ranging up to 93°C (200°F). More specifically, this invention relates to post-treating phosphoric acid anodized aluminum and its alloys to improve the corrosion-resistance and maintain adhesion bonding properties e.g. paint adhesion and the like. The trivalent chromium post-treatment (TCP) composition of this invention comprises an acidic aqueous solution having a pH ranging from 2.5 to 5.5 and preferably 2.5 to 4.5 or 3.7 to 4.0, and per liter of said acidic solution, from 0.01 to 22 grams of a water-soluble trivalent chromium compound, 0.01 to 12 grams of an alkali metal hexafluorozirconate, 0.0 to 12 or 0.001 to 12 grams of at least one fluorocompound selected from the group consisting of an alkali metal tetrafluoroborate, an alkali metal hexafluorosilicate and various combinations or mixtures thereof in any ratio, 0.001 to 10 grams of a water soluble divalent zinc compound, from 0 to 10 grams and preferable 0 to 2.0 grams of at least one water-soluble thickener, and from 0 to 10 and preferably 0 to 2.0 grams of at least one water-soluble non-ionic, cationic or anionic surfactant or wetting agent

It is therefore an object of this invention to provide an acidic aqueous solution comprising a trivalent chromium compound, an alkali metal hexafluorozirconate, and a tetrafluoroborate and/or hexafluorosilicate for treating phosphoric acid anodized aluminum and its alloys to maintain its adhesion and improve its corrosion-resistance characteristics.

It is another object of this invention to provide a stable acidic aqueous solution having a pH ranging from 2.5 to 5.5 which contains effective amounts of a trivalent chromium salt and a hexafluorozirconate for sealing phosphoric acid anodized aluminum and its anodized alloys.

It is a further object of this invention to provide a stable acidic aqueous solution having a pH ranging from 3.7 to 4.0 containing a trivalent chromium salt and a hexafluorozirconate for treating or sealing phosphoric acid anodized aluminum and its alloys at about room temperature and higher wherein said acidic solution contains substantially no hexavalent, chromium.

These and other objects of the invention will become apparent by reference to the detailed description when considered in conjunction with the accompanying Figs. 1-9 (photos).

### DESCRIPTION OF THE DRAWINGS

Fig. 1 is a photo of phosphoric acid anodized aluminum, 2024-T3 with no post treatment after exposure to 24 hours (1 day) of ASTM-B 117 neutral salt fog test.
Fig. 2 is a photo of phosphoric acid anodized 2024-T3 post treated with the composition of Example 5 (10 minute immersion at 24°C (75°F)) after exposure to 96 hours (4 days) of ASTM-B 117 neutral salt fog test.
Fig. 3 is a photo of a phosphoric acid anodized 2024-T3 post treated with the composition of Example 6 (10 minute immersion at 24°C (75°F)) after exposure to 96 hours (4 days) of ASTM-B 117 neutral salt fog test.
Fig. 4 is a photo of phosphoric acid anodized 2024-T3 post treated with the composition of Example 5 (10 minutes at 38°C (100°F)) after exposure to 1000 hours (42 days) of ASTM-B 117 neutral salt fog test.
Fig. 5 is a photo of a phosphoric acid anodized 2024-T3 post treated with the composition of Example 7 (10 minutes at 38°C (100°F)) after exposure to 1000 hours (42 days) of ASTM-B 117 neutral salt fog test.
Fig. 6 is a photo of a phosphoric acid anodized 2024-T3 post treated with the composition of Example 5 (40 minutes at ambient 24°C (75°F)) after exposure to 1000 hours (42 days) of ASTM-B 117 neutral salt fog test.
Fig. 7 is a photo of a phosphoric acid anodized 2024-T3 post treated with the composition of Example 7 (40 minutes at ambient 24°C (75°F)) after exposure to 1000 hours (42 days) of ASTM-B 117 neutral salt fog test.
Fig. 8 is a photo of a phosphoric acid anodized 2024-T3 post treated with the composition of Example 5 (5 minutes at 66°C (150°F)) after exposure to 1000 hours (42 days) of ASTM-B 117 neutral salt fog test.
Fig. 9 is a photo of a phosphoric acid anodized 2024-T3 post treated with the composition of Example 6 (5 minutes at 66°C (150°F)) after exposure to 1000 hours (42 days) of ASTM-B 117 neutral salt fog test.

### DETAILED DESCRIPTION OF THE INVENTION

More specifically, this invention relates to the process of using an acidic aqueous solution having a pH ranging from 2.5 to 5.5, and preferably from 2.5 to 4.5 or 3.7 to 4.0 for sealing phosphoric acid anodized aluminum and its alloys to maintain its adhesion bonding and to substantially improve the corrosion-resistance properties of the anodized aluminum(s). The process preferably comprises the use of an acidic solution comprising from 0.01 to 22 grams and preferably from 4.0 to 8.0 grams e.g. 6.0 grams of at least one water soluble trivalent chromium compound e.g. chromium sulfate, 0.01 to 12 grams and preferably 6.0 to 10 grams e.g. 8.0 grams of at least one alkali metal hexafluorozirconate, 0.0 to 12 or 0.001 to 12 grams and preferably 0.12 to 1.2 grams e.g. 0.24 to 0.36 grams of at least one fluorocompound selected from the group consisting of alkali metal tetrafluoroborates, alkali metal hexafluorosilicates and various mixtures or combinations thereof in any ratio, and from 0.001 to 10 grams and preferably 0.1 to 5.0 or 1.0 to 2.0 grams of at least one divalent zinc compound such as zinc sulfate.

In some processes, depending on the physical characteristics of the anodized aluminum e.g. the physical size of the anodized substrate, a feature is the addition of a thickener to the solution that aids in optimum film formation during spray and wipe-on applications by slowing down solution evaporation. This also mitigates the formation of powdery deposits that degrade paint adhesion. Moreover, the addition of thickeners, aids in proper film formation during large area applications and mitigates the diluent effect of rinse water remaining on the substrate during processing from previous steps. This additive yields films that have no streaks and have better coloration and corrosion protection. The water soluble thickeners such as the cellulose compounds are known and can be present in the acidic aqueous solution in amounts ranging from 0.0 to 10 grams and preferably from 0.0 to 2.0 grams and more preferably from 0.5 to 1.5 e.g., 1.0 gram per liter of the aqueous solution. Depending on the characteristics of the anodized aluminum, an effective but small amount of at least one water-soluble surfactant or wetting agent can be added to the acidic solution in amounts ranging from 0.0 to 10 grams and preferably from 0.0 to 2.0 grams and more preferably from 0.5 to 1.5 grams e.g. 1.0 grams per liter of the acidic solution. These water soluble surfactants or wetting agents are known in the prior art and are selected from the group consisting of non-ionic, cationic and anionic surfactants.

The trivalent chromium is added as a water-soluble trivalent chromium compound, preferably as a trivalent chromium salt. Specifically, in formulating the acidic aqueous solutions of this invention, the chromium salt can be added, conveniently, to the solution in its water soluble form wherein the valence of the chromium is plus 3. For example, some of the preferred chromium compounds can be prepared in solution in the form of Cr₂(SO₄)₃, (NH₄)Cr(SO₄)₂ or KCr₂(SO₄)₂ and any mixtures or combination of these compounds. The aluminum substrates are either phosphoric acid anodized aluminum or anodized aluminum alloys containing 60% or more by weight of aluminum. A preferred example of trivalent chromium concentration is within the range of 4.0 to 8.0 grams or 6.0 grams per liter of the aqueous solution. It has been found that particularly good results are obtained when the trivalent chromium compound is present in solution in these preferred ranges. The preferred metal fluorozirconate addition to the acidic solution ranges from 6.0 to 10 grams or 8.0 grams per liter of solution.

The treatment or sealing of the phosphoric acid anodized aluminum can be carried out at low temperatures e.g. about ambient or room temperature or at temperatures ranging up to 93°C (200°F). Room temperature treatment is preferred in that this eliminates the necessity for heating equipment. The seal coating may be air dried by any of the methods known in the art, for example, oven drying, forced air drying, exposure to infira-red lamps, and the like. For purposes of this invention, the terms phosphoric acid anodized aluminum and anodized aluminum alloys include aluminum and its alloys phosphoric acid anodized by methods known in the art.

In some treatments, the alkali metal tetrafluoroborates and/or hexafluorosilicates can be added to the acidic solution in amounts as low as 0.001 grams per liter up to the solubility limits of the compounds. For example, 50% weight percent of the fluorosilicate is added based on the weight of the fluorozirconate. In other words, for 8.0 grams per liter of the fluorozirconate salt, 4.0 grams per liter of fluorosilicate is added to the solution. For example, an alternative is to add 0.01 to 100 weight percent of the fluoroborate salt based on the weight of the fluorozirconate salt. Preferably, 1 to 10 weight percent e.g. 3% of the fluoroborate salt can be added based on the weight of the fluorozirconate salt. A specific example comprises 8.0 grams per liter of potassium hexafluorozirconate, 6.0 grams per liter of chromium III sulfate basic, 0.1 to 5.0 grams per liter of divalent zinc sulfate and 0.12 to 1.2 grams per liter of potassium tetrafluoroborate and/or hexafluorosilicate. An important result of the addition of the stabilizing additives i.e. fluoroborates and/or fluorosilicates is that the solution is stable while the pH is maintained between 2.5 and 5.5. However, in some cases the pretreatment solutions may require small adjustments to the pH by the addition of effective amounts of a dilute acid or base to maintain the pH in the range of 2.5 to 5.5 or lower e.g. from 3.25 to 3.5..

The composition or acid solution can also contain zinc compounds to further improve the corrosion protection of the phosphoric acid anodized coatings compared to compositions that do not contain divalent zinc compounds. The components of the solution are mixed together in water and can be used with no further chemical manipulation. The divalent zinc can be supplied by any chemical compound that dissolves in water at the required concentrations ranging from 0.001 to 10 grams and is compatible with the other components in the solution. Compounds that are particularly preferred include, for example, zinc acetate, zinc telluride, zinc tetrafluoroborate, zinc molybdate, zinc hexafluorosilicate, zinc sulfate and the like or any combination thereof in any ratio.

The following Examples illustrate the stable seal-coating solutions of this invention, and the method of using the solutions in maintaining the adhesion properties while improving the corrosion-resistance of phosphoric acid anodized aluminum and its alloys.

### EXAMPLE 1

### TCP5PZ2

A stable acidic aqueous solution having a pH ranging from 3.45 to 4.0 for post-treating phosphoric acid anodized aluminum and aluminum alloys to provide a corrosion-resistant and a color recognized coating thereon which comprises, per liter of solution, 3.0 grams of trivalent chromium sulfate basic, 4.0 grams of potassium hexafluorozirconate and 1.0 gram zinc sulfate.

### EXAMPLE 2

### TCPSB3

A stable acidic aqueous solution for post-treating phosphoric acid anodized aluminum and aluminum alloys to form a corrosion-resistant coating thereon which comprises, per liter of solution, 3.0 grams of trivalent chromium sulfate basic, 4.0 grams of potassium hexafluorozirconate, and 0.12 grams of potassium tetrafluoroborate.

### EXAMPLE 3

### TCP5B3Z4

A stable acidic aqueous solution for post-treating phosphoric acid anodized aluminum and aluminum alloys to provide a corrosion-resistant and a color recognized coating thereon which comprises, per liter of solution, 3.0 grams or trivalent chromium sulfate basic, 4.0 grams of potassium hexafluorozirconate, 0.12 grams of potassium tetrafluoroborate and 2.0 grams of divalent zinc sulfate.

Table 1 shows the corrosion ratings of three Examples for post-treating phosphoric acid anodized aluminum alloys of this invention in comparison to the composition of Example 2 coatings. Example 3 (TCP5B3Z4) and Example 1 (TCP5PZ2) on average had higher ratings.

**TABLE 1**

| Corrosion Resistance of Phosphoric Acid Anodize with Sealer on 2024-T3 Aluminum Alloy After 1,000 Hours of Exposure to ASTM B 117 Neutral Salt Spray | | | | | |
|---|---|---|---|---|---|
| | | | ***Immersion conditions*** | | |
| ***Applicable Patents*** | ***TCP Sealer composition*** | ***Ambient*/*10 minute*** | ***Ambient*/*40 minute*** | ***38°C* (*100F*)/*10-minute*** | ***66°C* (*150F*)/*5-minute*** |
| USP 6,500,532 | Example 2 5B3 | 0 | 6.7 | 5.7 | 3 |
| This Invention, USP 6,663,700, USP 6,669,764 | Example 3 5B3Z4 | 0 | 1 | 0 | 8 |
| This Invention, USP 6,663,700 , USP 6,669,764 | Example 1 5PZ2 | 0 | 7.7 | 7.7 | 6 |
| Note: Each rating is the average of 3 identically coated and exposed panels | | | | | |
| Corrosion rarings per ASTMD 1654 | | | | | |

### EXAMPLE 4

Add 3.0 grains per liter of chromium III sulfate basic and 4.0 grams per liter of potassium hexafluorozirconate to specific volume of deionized water. Maintain pH between 3.25 and 3.60 for 14 days using dilute potassium hydroxide or dilute sulfuric acid. After 14 days, adjust pH to 3.90 +1-0.05 and let sit overnight. Solution is ready to use.

### EXAMPLE 5

Add 3.0 grams per liter of chromium III sulfate basic, 4.0 grams per liter of potassium hexafluorozirconate, and 0.12 grams per liter potassium tetrafluoroborate to specific volume of deionized water. Let solution stand for approximately 10 days, or until pH rises to between 3.75 and 4.00. Solution is ready to use.

### EXAMPLE 6

To Example 4, add 1.0 grams per liter of zinc sulfate during initial mixing. Solution is ready to use.

### EXAMPLE 7

To Example 5, add 2.0 grams per liter of zinc sulfate during initial mixing. Solution is ready to use.

### EXAMPLE 8

Post treatment coatings were applied to anodized aluminum as follows. The phosphoric acid anodize process per ASTM D 3933, "Standard Practice for Preparation of Aluminum Surfaces for Structural Adhesives Bonding (Phosphoric Acid Anodizing)," was followed throughout. Immediately after anodizing 3" by 10" by 0.32" aluminum panels of 2024-T3 aluminum alloys by the Phosphoric Acid Anodize process, the panels were rinsed thoroughly two times in deionized water. Immediately after rinsing, the panels were immersed into a solution of either Example 6 or 7 for 10 minutes at ambient conditions. The immersion was immediately followed by two deionized water rinses. The panels were air-dried at ambient conditions before being subjected to neutral salt fog per ASTM B 117. The coupons were held in a rack at 15 degrees for the duration of the test. Control coupons of phosphoric acid anodized (PAA) not sealed were tested alongside the subject coatings.

Fig's.2 and 3 (photos) show the performance of post treatments from the compositions of Examples 5 and 6. Fig. 1 (photo) shows an unsealed PAA panel after exposure to ASTM B 117 neutral salt fog. The post treatments of Fig's. 2 and 3 provide improved corrosion resistance compared to the no post-treatment coating of Fig. 1.

### EXAMPLE 9

Test specimens were anodized as in Example 8. In this example, the compositions (solutions) from Examples 5 and 7 were heated to 38°C (100° Fahrenheit) and the panels were immersed for a total of 10 minutes. Fig's. 4 and 5 (photos) show corrosion performance of these coatings after 1000 hours of neutral salt fog per ASTM B 117. It is evident that the composition of example 7 is an improvement compared to the composition of Example 5.

### EXAMPLE 10

Test specimens were anodized as in Example 8. In this example, the compositions (solutions) from Examples 5 and 7 were kept at ambient conditions, 24°C (75° Fahrenheit) and the panels were immersed for a total of 40 minutes. Fig's. 6 and 7 (photos) show the improved corrosion resistance of these coating after 1000 hours of neutral salt fog per ASTM B 117.

### EXAMPLE 11

Test specimens were anodized as in Example 8. In this example, the compositions (solutions) from Examples 5 and 6 were heated to 66°C (150° Fahrenheit), and the panels were immersed for a total of 5 minutes. Fig's. 7 and 8 (photos) show the corrosion resistance of these coatings after 1000 hours of neutral salt fog per ASTM B 117.

Table 2 compares the corrosion resistance results of the Examples based on numerical ratings from ASTM D 1654. In the ASTM rating method, the best possible score is 10, meaning substantially no corrosion is evident on the test panel. Ratings decrease to 1, which represents substantially 100% corrosion of the panel surface. From the data in Table 2, it is evident that the process of this invention is an improvement over previous processes used for post treating or sealing phosphoric acid anodized aluminum and its alloys.

**TABLE 2**

| Numerical corrosion ratings of the panels treated with the compositions (solutions) and the process of this invention, based on ASTM D 1654, had ratings as high as 10 (no corrosion) to a low of 1 (fully corroded) where there was no post-treatments. The ratings comprise an average of three rated panels for each condition. | | | | |
|---|---|---|---|---|
| ***Compositions in Aqueous Acidic Solution*** | ***PROCESS CONDITlON*** | | | |
| | ***Ambient temperature 24°C (75°F) and 10 minute immersion (Example 8)*** | ***Ambient temperature 24°C (75°F) and 40 minute immersion (Example 10)*** | ***38°C 100°F and 10 immersion (Example 9)*** | ***66°C 105°F and 5 minute immersion (Example 11)*** |
| Control (no post treatment) | 0 after 24 hours | NA | NA | NA |
| example 5 | NA | 6.7 after 1000 hours NSF | 5.7 after 1000 NSF | 3 after 1000 hours NSF |
| Example 6 | after 96 hours NSF | 7.7 after 1000 hours NSF | hours 7.7 after 1000 hours NSF | 6 after 1000 hours NSF |
| Example 7 | 0 after 96 hours NSF | 1 after 1000 hours NSF | 0 after 1000 hours NSF | 8 after 1000 hours NSF |

For purposes of this invention, the water soluble surfactants or wetting agents can be added to the trivalent chromium solutions in amounts ranging from 0 to 10 grams per liter and preferably 0.5 to 1.5 grams per liter of the trivalent chromium solution. The surfactants are added to the aqueous solution to provide better wetting properties by lowering the surface tension thereby insuring complete coverage, and a more uniform film on the coated substrate. The surfactants include at least one water soluble compound selected from the group consisting of the non-ionic, anionic, and cationic surfactants. Some known water soluble surfactants having the solubility at the required concentrations include the monocarboxyl imidoazoline, alkyl sulfate sodium salts (DUPONOL®), tridecyloxy poly(alkyleneoxy ethanol) ethoxylated or propoxylated alkyl phenol (IGEPAL®), alkyl sulfonamides, alkaryl sulfonates, palmitic alkanol amides (CENTROL®), octylphenyl polyethoxy ethanol (TRITON®), sorbitan monopalmitate (SPAN®), dodecylphenyl polyethylene glycol ether e.g. TERGITROL®, alkyl pyrrolidone, polyalkoxylated fatty acid esters, alkylbenzene sulfonates and mixtures thereof. Other known water soluble surfactants include the alkyl phenol alkyloxylates, preferably the nonylphenol ethyloxylates, and the various anionic surfactants, having at least one sulfonate substituent in the phenyl ring, and the adducts of ethylene oxide with fatty amines. Other known water soluble compounds are found in "Surfactants and Detersive Systems", published by John Wiley & Sops in Kirk-Othmer's Encyclopedia of Chemical Technology, 3rd Ed.

When large surfaces do not permit immersion or where vertical surfaces are to be sprayed, thickening agents are added to retain the aqueous solution on the surface for sufficient contact time. The thickeners employed are known inorganic and organic water soluble thickeners which can be added to the trivalent chromium solutions in effective amounts e.g. a sufficient concentration ranging from 0 to 10 grams per liter and preferably 0.5 to 1.5 grams per liter of the acidic solution. Specific examples of some preferred thickeners include the cellulose compounds, e.g. hydroxypropyl cellulose (e.g. Klucel), ethyl cellulose, hydroxyethyl cellulose, hydroxymethyl cellulose, methyl cellulose and mixtures thereof. Some of the less preferred thickeners include the water soluble inorganic thickeners such as colloidal silica, clays such as bentonite, starches, gum arabic, tragacanth, agar and various combinations.

After preparing the surface to be treated via conventional phosphoric acid anodizing techniques, the solution can be applied by immersion, spray or wipe-on techniques. The solution also can be used at elevated temperatures up to 65°C and optimally applied by immersion to further improve the corrosion resistance of phosphoric acid anodize coatings. Solution dwell time is about 1 to 60 minutes, depending on the solution temperature and concentration of the solution. After dwelling, the remaining solution is then thoroughly rinsed from the substrate with tap or deionized water. No additional chemical manipulations of the deposited film are necessary for excellent performance. However, an application of a strong oxidizing solution can yield a film with improved corrosion resistance. The additional corrosion resistance is presumed to be due to the hexavalent chromium formed in the film from the trivalent chromium. The aqueous sealer composition may be sprayed from a spray tank apparatus designed to replace immersion tanks. This concept also reduces active chemical volume from 3785 ℓ (1,000 gallons) to 114 to 189 ℓ (30 to 50 gallons).

Another feature of this invention is the ability of this protective seal coating to provide the phosphoric acid anodized coatings with corrosion resistance better or at least equivalent to other known sealed anodic coatings produced with sulfuric, chromic, boric-sulfuric, or other known compositions. This capability has not been available before and offers new potential applications for phosphoric acid anodized in corrosive environments that were not previously possible. Phosphoric acid anodized aluminums have a major advantage over these other coatings in that its coating weights are typically 10 to 50 times lower. This yields significant weight savings and lower fatigue debit to structural aluminum alloys. In addition, this invention has the ability to enhance the performance of phosphoric acid anodize coatings currently being implemented as an adhesive bonding alternative to chromic acid anodizing. Phosphoric acid anodize coatings that have not been post treated are known to have inferior corrosion resistance, but are known also to have excellent bonding characteristics. This invention increases the corrosion performance of the anodized aluminums, while maintaining the adhesive bonding strength of the coatings. The terms, for purposes of this invention, "solubility" and "water soluble" mean water solubility of the chemical compounds used in the solutions of this invention at least at the concentrations set-forth herein.

## Claims

1. Process for sealing phosphoric acid anodized aluminium and aluminium alloys to improve the corrosion resistance and maintain the adhesive bonding strength which comprises treating the anodized aluminium and its alloys with an acidic aqueous solution having a pH ranging from 2.5 to 5.5; said acidic aqueous solution comprising, per liter of solution, from 0.01- to 22 grams of a trivalent chromium compound, 0.01 to 12 grams of an alkali metal hexafluorozirconate, 0.0 to 12 grams of at least one fluorocompound selected from the group consisting of an alkali metal tetrafluoroborate, an alkali metal hexafluorosilicate and mixtures thereof, from 0.001 to 10 grams of at least one divalent zinc compound, from 0.0 to 10 grams of at least one water soluble thickener and from 0.0 to 10 grams of at least one water- soluble surfactant.

2. The process of claim 1, wherein the pH of the acidic aqueous solution ranges from 3.7 to 4.0 and the temperature of the acidic aqueous solution ranges from ambient to 93°C (200°F).

3. The process of claim 1, wherein the trivalent chromium is a water soluble compound ranging from 4.0 to 8.0 grams, the alkali metal hexafluorozirconate is a water soluble compound ranging from 6.0 to 10 grams, and the fluorocompounds are water soluble compounds ranging from 0.12 to 1.2 grams.

4. The process of claim 1, wherein the thickener ranges from 0.5 to 1.5 grams and the surfactant ranges from 0.5 to 1.5 grams.

5. The process of claim 1, wherein the fluorocompound is present in the acidic aqueous solution in an amount ranging from 0.24 to 0.36 grams and the treated anodized aluminium is subsequently washed with water at temperatures ranging up to 93°C (200°F).

6. The process of claim 1, wherein the thickener is a cellulose compound present in the acidic aqueous solution in amounts ranging from 0.5 to 1.5 grams per liter.

7. The process of claim 1, wherein the trivalent chromium compound is trivalent chromium sulfate.

8. The process of claim 1, wherein the alkali metal hexafluorozirconate is potassium hexafluorozirconate.

9. The process of claim 1, wherein the trivalent chromium compound is trivalent chromium sulfate ranging from 4.0 to 8.0 grams, the alkali metal hexafluorozirconate is potassium hexafluorozirconate ranging from 6.0 to 10 grams, and the alkali metal tetrafluoroborate or alkali metal hexafluorosilicate ranges from 0.24 to 0.36 grams.

10. The process of claim 1, wherein the divalent zinc compound is at least one of a zinc acetate and a zinc sulfate.

11. The process of claim 1, wherein the water soluble surfactant is selected from the group consisting of water soluble non-ionic, anionic and cationic surfactants.

12. The process of claim 10, wherein the zinc sulfate is present in the aqueous solution in an amount ranging from 0.1 to 5.0 grams.

13. The process of claim 1, wherein the trivalent chromium compound is chromium sulfate present in the aqueous solution in an amount ranging from 4.0 to 8.0 grams, the mixture of alkali metal tetrafluoroborate and alkali metal hexafluorosilicate are present in the aqueous solution in an amount ranging from 0.001 to 12 grams.

## Patentansprüche

1. Verfahren zum Versiegeln von mit Phosphorsäure anodisiertem Aluminium und Aluminiumlegierungen um die Korrosionsbeständigkeit zu verbessern und die Klebefestigkeit zu erhalten, umfassend Behandeln des anodisierten Aluminiums und dessen Legierungen mit einer sauren wässrigen Lösung, die einen pH in einem Bereich von 2,5 bis 5,5 hat, wobei die saure wässrige Lösung pro Liter Lösung von 0,01 bis 22 Gramm einer dreiwertigen Chromverbindung, von 0,01 bis 12 Gramm eines Alkalimetallhexafluorzirkonats, von 0,0 bis 12 Gramm wenigstens einer Fluorverbindung ausgewählt aus der Gruppe bestehend aus einem Alkalimetalltetrafluorborat, einem Alkalimetallhexafluorsilikat und Mischungen davon, von 0,001 bis 10 Gramm wenigstens einer zweiwertigen Zinkverbindung, von 0,0 bis 10 Gramm wenigstens eines wasserlöslichen Verdickungsmittels und von 0,0 bis 10 Gramm wenigstens eines wasserlöslichen Tensids umfasst.

2. Verfahren nach Anspruch 1, wobei der pH der sauren wässrigen Lösung in einem Bereich von 3,7 bis 4,0 liegt und die Temperatur der sauren wässrigen Lösung in einem Bereich von Raumtemperatur bis 93 °C (200 °F) liegt.

3. Verfahren nach Anspruch 1, wobei das dreiwertige Chrom eine wasserlösliche Verbindung in einem Bereich von 4,0 bis 8,0 Gramm ist, das Alkalimetallhexafluorzirkonat eine wasserlösliche Verbindung in einem Bereich von 6,0 bis 10 Gramm ist und die Fluorverbindungen wasserlösliche Verbindungen im Bereich von 0,12 bis 1,2 Gramm sind.

4. Verfahren nach Anspruch 1, wobei das Verdickungsmittel in einem Bereich von 0,5 bis 1,5 Gramm liegt und das Tensid in einem Bereich von 0,5 bis 1,5 Gramm liegt.

5. Verfahren nach Anspruch 1, wobei die Fluorverbindung in der sauren wässrigen Lösung in einer Menge in einem Bereich von 0,24 bis 0,36 Gramm vorhanden ist und das behandelte anodisierte Aluminium nachfolgend mit Wasser bei Temperaturen in einem Bereich von bis zu 93 °C (200 °F) gewaschen wird.

6. Verfahren nach Anspruch 1, wobei das Verdickungsmittel eine Celluloseverbindung ist, die in der wässrigen Lösung in Mengen in einem Bereich von 0,5 bis 1,5 Gramm pro Liter vorhanden ist.

7. Verfahren nach Anspruch 1, wobei die dreiwertige Chromverbindung dreiwertiges Chromsulfat ist.

8. Verfahren nach Anspruch 1, wobei das Alkalimetallhexafluorzirkonat Kaliumhexafluorzirkonat ist.

9. Verfahren nach Anspruch 1, wobei die dreiwertige Chromverbindung dreiwertiges Chromsulfat in einem Bereich von 4,0 bis 8,8 Gramm ist, das Alkalimetallhexafluorzirkonat Kaliumhexafluorzirkonat in einem Bereich von 6,0 bis 10 Gramm ist und das Alkalimetalltetrafluorborat oder Alkalimetallhexafluorsilikat in einem Bereich von 0,24 bis 0,36 Gramm liegt.

10. Verfahren nach Anspruch 1, wobei die zweiwertige Zinkverbindung wenigstens eine von Zinkacetat und Zinksulfat ist.

11. Verfahren nach Anspruch 1, wobei das wasserlösliche Tensid ausgewählt ist aus der Gruppe bestehend aus wasserlöslichen nichtionischen, anionischen und kationischen Tensiden.

12. Verfahren nach Anspruch 10, wobei das Zinksulfat in der wässrigen Lösung in einer Menge in einem Bereich von 0,1 bis 5,0 Gramm vorhanden ist.

13. Verfahren nach Anspruch 1, wobei die dreiwertige Chromverbindung Chromsulfat ist, das in der wässrigen Lösung in einer Menge in einem Bereich von 4,0 bis 8,0 Gramm vorhanden ist und die Mischung aus Alkalimetalltetrafluoroborat und Alkalimetallhexafluorosilikat in der wässrigen Lösung in einer Menge in einem Bereich von 0,001 bis 12 Gramm vorhanden ist.

## Revendications

1. Procédé d'étanchéification d'aluminium anodisé à l'acide phosphorique et d'alliages d'aluminium pour améliorer la résistance à la corrosion et maintenir la force de liaison par collage, le procédé comprenant un traitement de l'aluminium anodisé et de ses alliages avec une solution aqueuse acide ayant un pH compris dans une plage allant de 2,5 à 5,5 ; ladite solution aqueuse acide comprenant, par litre de solution, de 0,01 à 22 grammes d'un composé de chrome trivalent, de 0,01 à 12 grammes d'un hexafluorozirconate de métal alcalin, de 0,0 à 12 grammes d'au moins un composé fluoré sélectionné dans le groupe constitué par un tétrafluoroborate de métal alcalin, un hexafluorosilicate de métal alcalin et un mélange de ceux-ci, de 0,001 à 10 grammes d'au moins un composé de zinc divalent, de 0,0 à 10 grammes d'au moins un épaississant soluble dans l'eau et de 0,0 à 10 grammes d'au moins un surfactant soluble dans l'eau.

2. Procédé selon la revendication 1, dans lequel le pH de la solution aqueuse acide est compris dans une plage allant de 3,7 à 4,0 et la température de la solution aqueuse acide comprise dans une plage allant de la température ambiante à 93°C (200 °F).

3. Procédé selon la revendication 1, dans lequel le chrome trivalent est un composé soluble dans l'eau compris dans une plage allant de 4,0 à 8,0 grammes, l'hexafluorozirconate de métal alcalin est un composé soluble dans l'eau compris dans une plage allant de 6,0 à 10 grammes, et les composés fluorés sont des composés solubles dans l'eau compris dans une plage allant de 0,12 à 1,2 grammes.

4. Procédé selon la revendication 1, dans lequel l'épaississant est compris dans une plage allant de 0,5 à 1,5 grammes et le surfactant est compris dans une plage allant de 0,5 à 1,5 grammes.

5. Procédé selon la revendication 1, dans lequel le composé fluoré est présent dans la solution aqueuse acide dans une quantité allant de 0,24 à 0,36 grammes et l'aluminium anodisé traité est ensuite lavé à l'eau à des températures allant de la température ambiante à 93 °C (200 °F).

6. Procédé selon la revendication 1, dans lequel l'épaississant est un composé de cellulose présent dans la solution aqueuse acide dans une quantité allant de 0,5 à 1,5 grammes par litre.

7. Procédé selon la revendication 1, dans lequel le composé de chrome trivalent est du sulfate de chrome trivalent.

8. Procédé selon la revendication 1, dans lequel l'hexafluorozirconate de métal alcalin est de l'hexafluorozirconate de potassium.

9. Procédé selon la revendication 1, dans lequel le chrome trivalent est du sulfate de chrome trivalent compris dans une plage allant de 4,0 à 8,0 grammes, l'hexafluorozirconate de métal alcalin est de l'hexafluorozirconate de potassium compris dans une plage allant de 6,0 à 10 grammes, et le tétrafluoroborate de métal alcalin ou l'hexafluorosilicate de métal alcalin est compris dans une plage allant de 0,24 à 0,36 grammes.

10. Procédé selon la revendication 1, dans lequel le composé de zinc divalent est au moins un d'un acétate de zinc et d'un sulfate de zinc.

11. Procédé selon la revendication 1, dans lequel le surfactant soluble dans l'eau est sélectionné dans le groupe constitué par des surfactants non ioniques, des surfactants anioniques et des surfactants cationiques solubles dans l'eau.

12. Procédé selon la revendication 10, dans lequel le sulfate de zinc est présent dans la solution aqueuse dans une quantité allant de 0,1 à 5,0 grammes.

13. Procédé selon la revendication 1, dans lequel le composé de chrome trivalent est du sulfate de chrome présent dans la solution aqueuse dans une quantité allant de 4,0 à 8,0 grammes, le mélange de tétrafluoroborate de métal alcalin et d'hexafluorosilicate de métal alcalin sont présents dans la solution aqueuse dans une quantité allant de 0,001 à 12 grammes.
